

## UNITED STATES PATENT OFFICE

2,599,397

INSOLUBILIZING AND SOLIDIFYING FATTY  
ACID ESTERS OF ALCOHOLS

Max Kronstein, New York, N. Y.

No Drawing. Application June 17, 1948,  
Serial No. 33,676

19 Claims. (Cl. 260—406)

1

This invention relates to a process for the solidification of fatty acid esters of alcohols, resins and resinous polyhydric alcohols, the first-mentioned being generally known as lipids, oils, fats, waxes, glycol esters and the like, which comprises treating said compounds with a particular class of potentially oxygen-yielding compounds known as per compounds, whereby a solidified product is obtained which is to a high degree insoluble in the usual petroleum and coal tar solvents and which can be readily purified without causing such a degree of swelling that the solid particles stick together in the form of a coherent gel.

It has been assumed that oils, fats, etc., exist only in the form of viscous liquids or in a resinous condition and that upon heating, with or without the use of chemicals and gases, a process takes place which increases their viscosity in a slowly progressing manner. Thus, oils which have undergone such treatment have been described as bodied oils, blown oils and the like, their viscosity being expressed by symbols such as Z-2, G, etc. This increasing degree of viscosity has also been expressed as an indication of changing molecular weight. Such compounds are generally found, prepared and used in a condition where it is possible to dissolve them in solvents by the application of heat or under decomposition in an attempt to obtain a stable solution.

It has also been assumed that upon continuous heating or upon chemical treatment, such compounds undergo partial insolubilization and result in a coherent sticky mass which is described as being gelatinized. Thus, fixed oils generally require an extended heating period at high temperatures (around 260° C.) before they achieve an at least partial insoluble or gelatinous phase. Gelatinous masses are also obtainable by heating such oils and the like under vacuum and by distilling off the non-gelatinized components at temperatures around 200° C.

Moreover, it has also been assumed that such gelatinization could only be achieved if the initial fatty acid radicals were in a relatively high degree of unsaturation, and it has been necessary to remove, as by vacuum distillation, the saturated components of fixed oils, etc., having a relatively high saturated fatty acid content before gelatinization could be effected with success. It is also known that gelatinization of fixed oils, etc., with the possible exception of China-wood oil, is accomplished by a more or less substantial loss of material.

2

I have observed that such gelatinized substances are characterized by being in the form of a coherent mass wherein the various insolubilized components are swollen together with each other and enclose the non-insolubilized components into a coherent, unitary mass. I have further observed that it is impossible to identify the individual insolubilized components from each other under the passing of light therethrough in a standing, moving or mixing state. I have also observed that these known gels are characterized in that the coherence of the components is great enough to allow substantial mechanical expansion of the gel without any evidence of the presence of individual, insolubilized particles. Even after the mechanical expansion has continued to a point where the gel substance is torn apart, the separated portions will again form a coherent mass upon being contacted by a mutual swelling liquid.

I have further observed that a small portion of the insoluble components eventually may be separated from the gel by repeated swelling of the gel with large excesses of solvent which results in a felling of minute amounts of the insoluble components. However, this laboratory method has not found any practical use other than to identify the presence of the insoluble components.

Accordingly, a broad object of my invention is to solidify oils, fats, waxes, resins, glycol esters, and other polyhydric alcohols esters, resinous polyhydric alcohols and the like directly from their initial state, from a modified state or from any state of increased viscosity such as blown or bodied oils, or an a state of dehydration or isomerization. More particularly, it is an object of my invention to effect this solidification directly within a short time, without forming a coherent gel and without substantial loss in weight between the beginning of the process and the occurrence of at least partial solidification.

A further object is to prepare an oil, wax, etc., base composition which can be readily insolubilized by the mere application of moderate heat.

A still further object is to prepare such a composition, adapted to be applied to a base, as by painting, dipping, spreading, spraying, impregnating, or by other known modes of application, in such manner that the coating can then be heated after being applied to the base and thereby be insolubilized and solidified directly onto the base.

55 Another object is to transfer the said oils, fats,

waxes, etc., into a state or condition wherein the components thereof no longer stick together after being insolubilized, whereby the insolubilized components can readily be obtained in a substantially odorless and tasteless condition. In this connection, it is still another object to prepare such insoluble products in a form where they may be made water soluble by enzyme activity or by combined enzyme and acid activity, even though such products are insoluble in the usual organic solvents and in water, whereby such products are adapted to be used as an article of food for animals and humans inasmuch as they are digestible in the living body of animals and humans.

Another object is to provide a process which will enable the ready separation of the insolubilized components of the said compounds from the non-insolubilized components whereby to eliminate the latter components which may impart unfavorable taste, odor or other undesirable characteristics to said compositions.

Another object is to provide a physical process whereby the novel compositions forming a part of this invention may be contacted with suitable solvents or swelling liquids in such manner that the various components of the composition do not stick in cohesive fashion, but can be readily separated in either a liquid or solid state without substantial mechanical effort.

A further object is to provide a process for producing the said solidified and insolubilized compositions forming a part of the present invention, which will be capable of having their color, swelling characteristics, chemical characteristics, and the like, be altered or varied.

Another object is to provide a process whereby oils, fats, waxes and the like which normally exist at room temperatures in more or less solid form or semi-solid form and which normally can be readily melted upon heating and again returned to their original solid or semi-solid state upon cooling, into a non-melting, solid form by use of the present solidification process.

Another object is to provide a process whereby the said fats, oils, waxes and the like, may be transferred into a novel physical state such that solidification and insolubilization thereof may be readily controlled to the desired extent by controlling the amount of heat and the length of heating time as well as the intensity of the heat.

Another object is to provide a process whereby the novel solidification method of the present invention may be controlled so as to permit the solidification to take place in a single or a selected plurality of operations which can take place at widely separated intervals.

Thus, it is an object of the invention to provide a process which will permit an initial, preliminary treatment which will enable a finer uniform form solidification to occur readily in a desired manner.

Another object is to provide a process whereby oils, fats, waxes, etc., which are partially or completely saturated and normally known as non-drying or slow-drying oils and the like, may be readily and completely solidified and insolubilized.

Another object is to provide a process whereby oils, fats, waxes, etc., may readily be purified or separated into components which are capable of being insolubilized on the one hand, and those components on the other hand which are incapable of being insolubilized.

Another object of the invention is to provide the foregoing novel compositions and products

resultant from use and application of the foregoing processes.

With these and other objects in view, which will be understood as the specification proceeds, I have discovered a method of insolubilizing and solidifying fatty acid esters of alcohols which comprises treating said esters with a potentially, free oxygen-yielding compound incapable of forming a metal soap with said esters, at a temperature sufficiently elevated to effect release of said free oxygen in said esters whereby to form a solidified composition which is insoluble in coal tar and petroleum solvents, and which is incapable of being melted without decomposition in the absence of contact with an additional compound, particularly metal soaps of fatty acids.

The compounds and compositions which may be physically altered by virtue of the present process generally include oils, fats, waxes, resins, glycol esters of fatty acids, or partial glycol esters of fatty acids, resinous polyhydric alcohols and the like which, for convenience of the chemist, may be identified as esters or partial esters of fatty acids and mono-hydric alcohols, di-hydric alcohols and other polyhydric alcohols. Thus, in the case of polyhydric alcohol esters of fatty acids, one or more of the hydroxy groups of the alcohols may be replaced or esterified with a fatty acid radical whereas the remainder of the hydroxy groups may remain unaltered or may be replaced by other radicals. Examples of the latter include alkyd resins which are partial fatty acid esters of polyhydric alcohols wherein at least one of the hydroxy groups has been esterified with a phthalic anhydride radical. Other examples include resinous polyhydric alcohols wherein at least one of the hydroxy groups of the polyhydric alcohols has been replaced by an oxy-aryl radical, such as an oxy-benzene radical or the like.

By further way of example it should be pointed out that the invention is also applicable to partial esters of the type which contain hydroxy groups, such as di-stearin and mono-stearin. In this connection, it is also desired to point out that the present invention is equally applicable to saturated and partially saturated fatty acid radicals as well as to unsaturated fatty acid esters of the hydroxy alcohols, both monohydric and polyhydric.

The particular potentially, free oxygen-yielding catalysts compounds which may be reacted with the said oils, fats, etc., to obtain the solidified and insolubilized compounds and compositions of the present invention may comprise either hydrogen peroxide or organic per compounds of a lipophylic, oil-soluble character. One requirement of these catalysts is that they be capable of releasing active oxygen in such a free state and in such a manner that the free oxygen is capable of acting as a catalytic agent in promoting the transformation of the initial oils, fats, waxes, etc., into a solid, insoluble, non-melting state. A further requirement of the organic, potentially oxygen-yielding peroxide catalysts is that they be oil-soluble or lipophylic in character; that is, that they have a greater affinity for lipids generally than they do for water, and as such they must be capable of being uniformly distributed in the initial starting compounds which are thereby solidified and insolubilized. Perhaps the most important requirement of the potentially, free oxygen-yielding catalyst compounds is that they be incapable of forming a metal soap. By metal soap I mean to include any metal compound

of an organic acid or ester thereof which is at least partially soluble in a fatty acid ester of an alcohol.

It is surprising indeed that hydrogen peroxide may be successfully used in the practice of the invention in view of its hydrophylic character, but I have found that by maintaining the reaction temperature near, at or above the boiling point of the hydrogen peroxide, I am able to effect the transformation by repeating the action one or more times. I have also found that continual stirring of the reacting mass contributes appreciably to the transformation reaction. While I do not desire to be restricted to any particular theory, it is my observation that this water of the  $H_2O_2$  boils off during the transformation before it can hinder the catalytic action of the free, active oxygen.

The organic, potentially oxygen-yielding catalyst compounds are generally of the alkyl, aryl, and alkyl aryl peroxide type which are of an oil-soluble or lipophylic character. Thus, I have selected certain specific catalysts which are representative of the class of catalyst compounds which come within the purview of my invention. These include

Diacetyl peroxide,  
Tertiary butyl perbenzoate,  
Di-tertiary butyl peroxide,  
Tertiary butyl hydroperoxide,  
Benzoyl peroxide, and  
Dimethyl benzyl hydroperoxide (cumene hydroperoxide).

Likewise, oxygen-yielding, organic per compounds which are more lipophylic than hydrophylic in character are operable; whereas, compounds which are both hydrophylic and lipophylic in a state of balance are generally operable under more extreme conditions of heat, excess amount of catalyst, time of reaction and repetitions of the present process. Moreover, I have found that ordinary metallic peroxides, such as magnesium peroxide are not operable because they result in the formation of a metallic soap which, according to my discoveries as set forth in my copending application, Ser. No. 748,665, now Patent 2,476,879, issued July 19, 1949, causes the solubilization and liquefaction of the compounds treated.

Moreover, I have found that the efficiency of the transformation and the uniformity of the product can be increased by adding to either the initial compound or the catalyst or both, an additional compound which is a solvent for either the initial compound and/or the catalyst. Thus, I have found it advantageous to add one part toluene to two parts tertiary butyl perbenzoate catalyst. By way of further example, 7 parts dimethyl phthalate may be added to three parts di-acetyl peroxide. In this connection, it has been found desirable to select a catalyst of the above type, the boiling point of which is in the neighborhood of the reaction temperature at which the catalyst is especially effective in releasing the free oxygen, whereby the presence of the added solvent serves to intensify the solidification.

The solidification which takes place actually produces a solid state in contrast to the known state of gelatinization. The invention is as equally applicable to natural or synthetically produced non-gelatinized compositions as it is to partially and completely gelatinized compositions. However, in the latter case, I have found

by actual experiment that a higher percentage of insoluble matter is produced although it appears to be developed within and closely adjacent to the gelatinous portions. Thus, I have found that the separation of the insolubilized, solidified portion from the non-solidified portion of the partially or completely gelatinous mass is rendered more difficult. Accordingly, I have found that it requires repeated and extended separation steps to achieve an actual yield which is equal to the percentage of solidification that has taken place within the gelatinous mass.

The following working examples will serve to illustrate the processes and products coming within the realm of the present invention and will also serve to illustrate the use of a representative number of the class of initial starting compounds and compositions, potentially, free oxygen-yielding catalysts, solvents, and solidified and insolubilized products covered by the present invention:

*Example 1*

About 500 parts linseed oil were mixed with 25 parts toluene solvent and 50 parts t-butyl-perbenzoate catalyst and slowly heated. When the first gas-bubbles began to develop at the bottom of the container, the heating was continued under stirring. When the temperature reached about 125° C., the heat source was shut off and stirring was continued. The temperature continued to rise during the gas development. When it had reached about 150° C., the mass solidified to a fluffy substance which was raising in the kettle. The temperature continued rising until the reaction had come to an end at which time the reaction product had solidified. The product also may be obtained without the addition of solvent and without stirring of the mixture during the transformation.

It has been found helpful in observing the course of the reaction, to drop a small sample of the compound on a hot place to indicate the formation of the non-melting, solid product. After solidification, further heat development can be broken up by stirring cold air into the solidified substance or by transferring the solid substance into a cold, neutral liquid. The product of this process is in form of a solid, fluffy or poppy substance which will not melt without decomposition. It does not dissolve in toluene, benzoyl, petroleum naphtha or any of the usual solvents for fixed oils. It swells to such a degree that it increases its volume in contact with solvents, but does not swell in such manner or to such extent that a coherent swollen mass is obtained.

Accordingly, the resulting product can be purified from unused parts of the perbenzoate catalyst, or decomposition products, or from the non-solidified portion of the oil, by the use of said solvents, including boiling in such solvents or extraction with solvent vapours. The product can be filtered off and dried in an oven at temperatures around and above 50° C. It can also be boiled in water and then dried in an oven, or it can be dried at room temperature over desiccator substances. The product can likewise be purified by boiling in water and then treating with organic solvents. These purification treatments can be repeated until the desired state of isolation of the insoluble product and the desired conditions of taste and odor have been reached.

In heating the solid substance in an oven at about 55° C. for an extended period, or at about 100° C for a shorter period, a certain modifica-

tion can be obtained, whereby the solidified product darkens or appears more intense in color. It has been observed that such modification substantially ceases at a certain point and thereafter further heating for 48 hours at 100° C. does not appreciably modify the product.

While preferred heating temperatures for the various stages of treatment of purification and drying are set forth in the examples, it will be understood that temperatures will vary in accordance with the physical and chemical condition of the starting materials, the quantities of the starting materials and other substances employed, and the form and the speed of heating.

#### Example 2

The process set forth in Example 1 was practiced with the following materials:

| Oil Used                                                            | Source of Free Oxygen                                                         | Added Volatile Solvent |
|---------------------------------------------------------------------|-------------------------------------------------------------------------------|------------------------|
| (a) 100 parts China wood oil.                                       | 8 parts t-butyl perbenzoate.                                                  | -----                  |
| (b) 53 parts Florida tung oil.                                      | 4 parts d-tertiary-butyl peroxide.                                            | 25                     |
| (c) 120 parts soybean oil with 5 parts rosin.                       | mixture of 9 parts t-butyl perbenzoate with 4.5 parts t-butyl-hydro-peroxide. | -----                  |
| (d) 20 parts linseed oil (break stabilized) with 10 parts tung oil. | 3 parts t-butyl perbenzoate.                                                  | -----                  |
| (e) 80 parts perilla oil with 20 parts China wood oil.              | 10 parts t-butyl-perbenzoate.                                                 | 30 5 parts benzol.     |
| (f) 26 parts linseed oil Z-2...                                     | 2.3 parts 95% benzoyl peroxide with stearic acid.                             | -----                  |

#### Example 3

The process set forth in Example 1 was followed in solidifying cottonseed oil, an oil of the group of semi-drying or non-drying oils. 44 parts cottonseed oil were mixed with 2 parts toluene and 4.8 parts t-butyl-perbenzoate and heated as set forth in Example 1. Gas development occurred especially between 150 and 200° C. After the reaction had quieted down, the oil had become more viscous than it was before the treatment, but it had not yet been solidified.

The ultraviolet spectrum of the oil in this modified condition showed a clear shifting in optical density. The modified oil also had a higher viscosity and lower iodine number than the initial oil.

After repeating the reaction on the modified oil with an additional 3 parts of the same catalyst, solidification was obtained at about 140° C. in the same manner as the drying oils of Examples 1 and 2. The solidified substance was purified by immersing it into petroleum ether for 15 minutes, decanting the ether, and repeating the extraction. After filtering, the solid substance was pressed against a porous filter paper, washed again with petroleum ether and dried. Then it was further purified by heating it with water and again dried. A loose and light colored solid substance was obtained with a very slight degree of odor or taste which can be removed by further extraction.

#### Example 4

The process set forth in Example 1 was followed in solidifying cottonseed oil. The oil was first treated by distilling off the oily substance. In this particular example, 19% of the substance of the oil was removed by vacuum distillation and a clear oil was obtained. The clear oil was treated as set forth in Example 1, by mixing 44 parts of

the modified cottonseed oil product with 2 parts petroleum naphtha and 2.5 parts t-butyl-perbenzoate. In heating it as set forth in Example 1, the substance was solidified in one treatment between, about and above 135 and 200° C.

#### Example 5

The process of Example 1 was applied to corn oil, another semi-drying or non-drying oil, by treating it in the two steps as set forth in Example 3. 56 parts corn oil were treated initially with 5 parts, secondly with 3 parts t-butyl-perbenzoate, whereby solidification was obtained.

#### Example 6

This exemplifies the solidification of a semi-drying or non-drying oil together with a drying oil, whereby the solidification occurs more rapidly. 45 parts corn oil were mixed with 10 parts tung oil and 7 parts t-butyl-perbenzoate. They were heated in accordance with Example 1. Solidification occurred in the initial treatment between at about 135 to 175° C.

#### Example 7

The process set forth in Example 1 was applied to a plant wax; namely, carnauba wax. 58 parts commercial carnauba wax were melted by heating to about 105° C. Seven parts t-butyl-perbenzoate were added as a source of free oxygen and the heating was continued. At about 130° C., gas development occurred and the temperature continued to rise, even after removal of the reaction vessel from the source. Solidification occurred freely at about 180° C. The solid product did not melt on a hot plate. It was purified by boiling it in about 4 times its own weight of toluene followed by hot filtering. The operation was repeated with toluene, again with petroleum ether, and after drying, again with ethyl alcohol, and finally boiled twice in water to remove all traces of decomposition products resulting from the catalyst treatment. A yield of about 45% insoluble product substance was obtained.

#### Example 8

Plant waxes generally require more than one treatment with the oxygen-yielding catalyst to achieve solidification, as shown by the following:

| Wax Used                                                          | Number of Treatments | Source of free oxygen                                                                                                                                                         |
|-------------------------------------------------------------------|----------------------|-------------------------------------------------------------------------------------------------------------------------------------------------------------------------------|
| (a) 25 grams Ouricuri wax                                         | 1                    | 3 g. t-butyl-perbenzoate heated up to about 185° C                                                                                                                            |
|                                                                   | 2                    | 2 g. of the same catalyst heated to solidification                                                                                                                            |
|                                                                   | 1                    | 3 g. t-butyl-perbenzoate heated up to about 170° C                                                                                                                            |
| (b) a plant wax derived from herbs or shrubs 25 g. Candelilla wax | 2                    | 2 g. of the same catalyst were added after the compound of the first treatment had been cooled to about 100° C. Some gel-formation occurred in addition to the solidification |
|                                                                   | 1                    | 4 g. t-butyl-perbenzoate caused, on heating up to 190° C, a vehement reaction whereby a gelatinous substance was formed which was cooled to about 110° C                      |
| (c) a plant wax derived from fruits and berries; 26 g. Japan wax  | 2                    | 2 g. of the same reagent were added and a solid substance was formed.                                                                                                         |

#### Example 9

In this example cod liver oil was used in producing a solid oil substance according to the proc-

ess set forth in Example 1. 40 parts cod liver oil were mixed with 1.5 parts benzoyl peroxide and heated under stirring at about 85° C. The solid source of oxygen appeared to go into a liquid combination with the oil, and on continuing the heating, the free oxygen was developed. The heating was continued to about 200° C. The clear modified oil was stored for several weeks and on heating it again with 2.5 parts t-butyl-perbenzoate, solidification occurred. As set forth in Example 4, the oil can be initially distilled to remove a portion of the nonsolidifiable components.

The same process was carried out with lard oil, solidification being obtained in the same manner.

#### Example 10

The process set forth in Example 1 was applied to a fish oil; namely, Menhaden fish oil. 40 parts of the oil were solidified in two steps with the same source of free oxygen, using a mixture of the oil with 2 parts xylene and 4 parts t-butyl-perbenzoate and heating it to about 200° C. After cooling the product to about 85° C., the substance was again treated with 3 parts of the same catalyst.

The oil was characterized after the first treatment by a change in viscosity, a decrease in the iodine number and a shift in the optical density in its ultraviolet absorption spectrum, in comparison to the same figures for the initial, untreated oil.

#### Example 11

The process set forth in Example 1 was applied to bacon fat, a fixed oil which has a solid appearance, at normal room temperatures. 30 grams commercial bacon were slowly heated so that the fat substance became liquified and could be separated from the non-fat substance. In this liquid form, the oil-like fat substance was decanted and, after cooling, a white fat was obtained. 20 grams of this white fat were mixed with 2 parts di-tertiary-butyl-di-perphthalate. One part toluene was added and the mixture heated to about 180° C. After cooling to about 70° C., the substance was heated with about 1.8 parts t-butyl-perbenzoate catalyst. Solidification occurred and the product was then purified by extracting the substance in a Soxleth extraction apparatus using a petroleum derived solvent as the purifying liquid. The purified substance consisted of loose, light solid particles of a slightly cream-colored appearance.

#### Example 12

The process set forth in Example 1 was applied to beeswax, an insect wax. 41 parts of commercial white beeswax were melted and mixed with 5 parts of t-butyl-perbenzoate. Gas development occurred vehemently on heating between 140 and 164° C., which continued after vessel was removed from the hot plate. No solidification having occurred, heating was continued up to about 200° C. Then the mass was allowed to cool to about 90° C. Again 4 parts of the same source of free oxygen was added and the heating procedure was repeated. Since solidification had not yet occurred, a third treatment with 4 parts of the same perbenzoate was carried out which resulted in solidification at about 170° C. The solid product was purified by extraction with toluene and, after drying, by boiling in water and drying at 115° C. for 5 hours. A yield of about 50% insoluble product was obtained.

#### Example 13

|    | Type of Wax                                               | Type of Catalyst                                                                                                                                                                                                                                                                                                                                                                                                                                                                 |
|----|-----------------------------------------------------------|----------------------------------------------------------------------------------------------------------------------------------------------------------------------------------------------------------------------------------------------------------------------------------------------------------------------------------------------------------------------------------------------------------------------------------------------------------------------------------|
| 5  | (a) 25 g. shellac wax, an insect wax.                     | 3 g. t-butyl-perbenzoate was utilized in each of three treatments. Solidification occurred at around 165° C. About 72.4% yield of solidified substance was obtained after purification.                                                                                                                                                                                                                                                                                          |
| 10 | (b) 25 g. woolfat of the type known as lanolin.           | 4 g. t-butyl-perbenzoate developed a very stormy reaction with strong heat development. Partial solidification occurred in the first treatment. After cooling, 3 g. of the same catalyst was added, followed by heating. When the reaction began, the vessel was removed from the heater and the temperature continued rising to above 205° C. The weight of the solid final product was not much different from the weight of the initial woolfat.                              |
| 15 | (c) 25 grams spermaceti wax.                              | Treated with 4 grams of t-butyl-perbenzoate. The composition was heated up to about 190° C. After cooling, 3 grams of the same catalyst were added which resulted in a violent reaction and the formation of a yellowish oily substance. After cooling, to about 120° C., 2.5 g. of the same catalyst was added. The composition was then heated to about 140° C., after which the temperature rose steadily to about 200° C. and the resulting product became fully solidified. |
| 20 |                                                           | The mixture was treated with 4 parts 95% benzoyl peroxide in stearic acid. The mixture was heated to above 200° C. and then cooled. Thereafter, 3 g. of the same catalyst were added, the reaction beginning at about 210° C. at which time the mass turned to a brownish solid.                                                                                                                                                                                                 |
| 25 | (d) 32 parts Florida Tung oil and 8 parts Candelilla Wax. |                                                                                                                                                                                                                                                                                                                                                                                                                                                                                  |
| 30 |                                                           |                                                                                                                                                                                                                                                                                                                                                                                                                                                                                  |

#### Example 14

25 grams powdered Montan wax were heated with 4 g. t-butyl-perbenzoate. The reaction began so violently around 120° C. that the vessel was removed from the source of heat. The temperature went up to about 185° C. and partial solidification occurred. After cooling to below 140° C., 0.5 g. more of the catalyst were added and solidification was obtained. The second test was discontinued at around 174° C. by throwing the reaction product into a solvent to interrupt the reaction. From the full purification in solvents and in water, about 28 to 30% solid insoluble, infusible substance was isolated at that point of the reaction.

#### Example 15

|    | Synthetic Oil                                                                                                  | Oxygen-yielding catalyst                                                                           | Volatile Solvent added       |
|----|----------------------------------------------------------------------------------------------------------------|----------------------------------------------------------------------------------------------------|------------------------------|
| 55 | (a) 92 parts isomerized linseed oil (commercial Isoline Z3).                                                   | 8 parts diacetyl peroxide.                                                                         | 16 parts dimethyl phthalate. |
| 60 | (b) 30 parts synthetic oil, obtained from combining sorbitol with soya fatty acids (commercial "Atlas G 876"). | 1.8 parts benzoyl peroxide.                                                                        | -----                        |
| 65 | (c) 40 parts of a synthetic oil from sorbitol and linseed fatty acids (commercial "Atlas G 875").              | 4 parts di-tertiary-butyl-diperphthalate (a solid that melts in the oil at about 75° C.).          | -----                        |
| 70 | (d) 33 parts of a linseed oil which was reacted with maleic anhydride (commercial "Trimol").                   | 1.5 parts di-tertiary-butyl-diperphthalate.                                                        | -----                        |
| 75 | (e) 42.5 parts dehydrated castor oil (commercial "Castung 403 Z3").                                            | 4 parts di-tertiary-butyl-diperphthalate.                                                          | 2 parts petroleum naphtha.   |
|    | (f) 40 parts dehydrated castor oil (commercial "Castung 403 Z3").                                              | 2 di-tertiary-butyl-peroxide. Solidification begins at 145° C., but temperature goes up to 195° C. | -----                        |
|    | (g) 30 parts synthetic triglyceride oil (commercial Neo fat 290).                                              | 3 parts t-butyl-perbenzoate.                                                                       | 2 parts petroleum naphtha.   |

## 11

In all above instances, solidification was achieved in accordance to the process set forth in Example 1.

## Example 16

This exemplifies the process of Example 1 as applied to a synthetic wax-like material solidified according to Example 1.

(a) 22 g. polyethylene glycol di-tri-ricinoleate were heated with 2 grams t-butyl-perbenzoate. In the first treatment a strong reaction occurred and solidification was reached between 150 and 170° C. The purification was performed in the same manner as hereinbefore set forth.

(b) The solidification of another product of a dihydric-stearate, an emulsifiable wax-like esterification product of a dihydric alcohol (like diethylenglycol) with a fatty acid, obtained under pressure and heat in the presence of a catalyst, e. g., sodium glycerophosphate, was successfully accomplished. In heating 30 parts of this ester with 3 parts t-butyl-perbenzoate up to 210° C., and a second time with the same amount of the reagent up to 200° C., no solidification occurred. After a third treatment with 2 parts of the reagent some solidification was produced above 150° C. and after a fourth treatment with about 2 parts of the catalyst rapid solidification of the ester resulted.

(c) In a similar way full effect was reached at the fourth treatment of 42 parts diethylene glycol monolaureate (Glaurin) with 4, 3, 3 and 2 parts of the t-butyl-perbenzoate respectively. Solidification occurred around 160° C. and the temperature rose to about 190° C. Purification was performed with the usual solvent treatment.

## Example 17

This exemplifies the application of the process set forth in Example 1 to such compounds which contain groups of polyhydroxyl alcohols and fatty acids with phthalic anhydride (commercial "alkyd" resins).

In this example the alkyd resin is used in a form wherein it has been modified with a drying oil. 150 parts of an alkyd resin of a long oil-modified group, obtained from polyhydroxyl alcohol and phthalic anhydride and soybean oil substance were mixed with 10 parts toluene and 14 parts t-butyl-perbenzoate and treated as set forth in Example 1 until solidification occurred. Solidification occurred quite rapidly.

## Example 18

This exemplified the application of the process of Example 10 to another group of alkyd resins which contain non-drying-oil substance instead of the drying oil substance of Example 10.

| Alkyd compound with non-drying oil                    | Oxygen-yielding Catalyst     | Added Volatile Solvent |
|-------------------------------------------------------|------------------------------|------------------------|
| (a) 41 parts "alkyd" resin (commercial "Rezyl 92-6"). | 5 parts t-butyl perbenzoate. | 5 parts toluene.       |

(The product obtained was well solidified, but still less uniform in character than the following examples.)

|                                         |                                                                                                       |                  |
|-----------------------------------------|-------------------------------------------------------------------------------------------------------|------------------|
| (b) 48 parts of the same alkyd resin.   | Treated initially with 3 parts benzoyl peroxide and, after cooling, with 3 parts t-butyl-perbenzoate. | 5 parts toluene. |
| (c) 16.5 parts of the same alkyd resin. | Two successive treatments with 1.5 parts t-butyl-perbenzoate.                                         | 11 parts xylene. |

## 12

## Example 19

The following embodiments exemplify modification of the rate of solidification in accordance with the processes as set forth above, such modification being accomplished by combining slower solidifying compounds with those which react more rapidly, or by modifying those which are solidified rapidly by combining them with others which react more slowly.

| Compounds for Solidification                                                     | Modifying Substance | Catalyst Oxygen Source         | Volatile Solvent Added |
|----------------------------------------------------------------------------------|---------------------|--------------------------------|------------------------|
| (a) 15.5 parts alkyd resin with soybean oil substance (commercial Aropiaz 1085). | None.               | 1.5 parts t-butyl-perbenzoate. | 5 parts toluene.       |

(Solidified rapidly in accordance with Example 1.)

|                                         |                           |                    |                 |
|-----------------------------------------|---------------------------|--------------------|-----------------|
| (b) 15.5 parts of the same alkyd resin. | 3.5 parts cottonseed oil. | Same as in (a).... | Same as in (a). |
|-----------------------------------------|---------------------------|--------------------|-----------------|

(Solidified somewhat more slowly than the previous example.)

|                                                                         |       |                                                                             |                  |
|-------------------------------------------------------------------------|-------|-----------------------------------------------------------------------------|------------------|
| (c) 16.5 parts alkyd resin with non-drying oil (commercial Rezyl 92-5). | None. | Two step treatment involving 1.8 parts and 1.2 parts catalyst respectively. | 11 parts xylene. |
|-------------------------------------------------------------------------|-------|-----------------------------------------------------------------------------|------------------|

(Solidified in two steps around 150 to 180° C.)

|                                                     |                         |                |  |
|-----------------------------------------------------|-------------------------|----------------|--|
| (d) 15 parts of the same alkyd with non-drying oil. | 3 parts China wood oil. | 1.8 parts..... |  |
|-----------------------------------------------------|-------------------------|----------------|--|

(Solidified in one step below 190° C.)

## Example 20

This example shows that the solidification products can be effected by enzymes and acids in the process of digestion.

In the course of the specification it has been pointed out that the insolubilized solidifications of these esters are insoluble in the usual solvents and in water. Thus, these stable and easily transportable materials can be used where, for instance, ordinary oils would be used, so long as it is not necessary to use such oils in liquid or soluble form. To demonstrate this, the present example shows that the insolubility of the solidified substance does not eliminate its digestibility and it shows that the solidified substances of the present invention are not basically different in this respect:

(A) Tests were made by actual feeding of the solidified substances to a living animal, a young white male rat of known background and of an initial weight of 219.3 grams. The feeding circle was begun after a 24 hours period of starving the animal with water supply exclusively. Each day afterwards, the animal received a food offering consisting of 2.5 g. dry solidified ester of changing origin made in accordance with the present invention and a mixture of 13 g. of the same solidification mixed with 20 g. scrambled raw egg substance. The weight of the intake and the content of insoluble substance in the excrements was checked in each case and the percentage of digested solids was calculated. The animal was

fed on subsequent days with solidifications of the following examples:

- (a) Example 1: Vegetable oil (linseed oil)
- (b) Mixture of 8 parts solids of Example 11: animal fat (bacon fat), with 5 parts solids of Example 9: animal oil (cod liver oil)
- (c) Example 12: Wax from animal source (beeswax)
- (d) Example 15: Synthetic triglyceride oil (Neo Fat 290)
- (e) Example 5: Vegetable non-drying oil (corn-oil)
- (f) Example 7: Plant-wax (carnauba wax)
- (g) Example 18: Oil-modified alkyd resin (Rezyl 92-5)

In all cases the animal took in daily between 10 and 15 g. of the solidification. In determining the amount of insoluble matter remaining in the excrements, the fact was neglected that even under normal kernel feeding conditions, the animal's excrements contain about 45% insoluble substance.

But even overlooking this fact, and deducting all insoluble substance in the excrements from these tests as undigested solidifications, the following results were obtained:

Average of digested substance from test *a* to *e* (between 53% and 74% for the various samples).

From test *f*—48.8% and test *g* 34.2%.

This gives an average of 54.5% for all tests which is not much different from the normal data on the usual food of the same animal. After test *g*, the weight of the animal was 215.2 g.

(B) In a second series the solidifications were first soaked in water for 24 hours before feeding and 2.5 g. bread was added to the daily diet for a more complete nourishment; the results were as follows:

- (h) Solids of Example 1
- (i) Solids of Example 10
- (k) Solids of Example 12

Based on 5 days' feeding, the percent of digested solids went up to 56.5 to 80.3% with an average of 67.3% and the weight of the animal rose to 228.5 g.

(C) At the end of the test series, mixtures of these water-soaked solidifications (1 part dry weight) with the normal kernel food (3 parts) were given, readily accepted and consumed.

The tests show that the solidifications are indeed digestible. The above solidifications were also eaten in small amounts by several humans and were digested in the normal manner, so far as is known, without ill effects.

#### Example 21

This exemplifies the application of the present process for the solidification and insolubilization of coatings, impregnations and other forms of layers produced from compounds containing polyhydroxyl alcohol-fatty acid esters, including such compounds which contain other ester-forming groups; that is, including, for instance, alkyds, being applied for the purpose of film-forming in a condition where they are combined with at least one thinning liquid.

50 parts of bodied linseed oil (Z-2) were mixed with 25 parts toluene. To this mixture, 5 parts tertiary butyl hydroperoxide in an oil-solvent mixture were added.

In another embodiment 5 parts tertiary butyl perbenzoate were added directly to the oil and

warmed slowly together at a temperature below that at which oxygen is released, the still soluble mixture being diluted with solvent.

These mixtures were stored for several months without any substantial influence on the stability of the mixture. However, upon heating the mixtures to a temperature permitting the release of oxygen and the partial escape of solvent, the solidification occurred as set forth in Example 1.

When parts of the mixture were spread over a base, as by coating on a panel, or by dipping a piece of metal in the mixture, an insolubilization was produced when such covered parts were exposed in a heated drying oven, or upon exposure to infra red light, or otherwise heated so that the free oxygen was released from the coating mixture after its application. It was found that the film had a higher percentage of insoluble substance than a similar film produced from the same initial oil and under the same conditions without utilizing the present catalysts (using similar film thickness, during temperature drying time, etc.).

The same process was also successfully applied to the remaining natural and synthetic initial compounds cited in the preceding examples.

#### Example 22

The oxygen-yielding substance itself may be used as a solvent for the compound which is to be applied and subsequently solidified. In accordance with this discovery, 50 parts of soybean oil were mixed with 6 parts butyl-hydroperoxide and treated like the coating compounds set forth in Example 21.

#### Example 23

Compounds containing phthalic anhydride compositions, in addition to the usual oils, may be insolubilized and solidified. 72 parts alkyd resin derived from a polyhydroxyl alcohol, phthalic anhydride and the substance obtained from dehydrated castor oil were mixed with 36 parts xylene solvent. 7 parts t-butyl-perbenzoate were added and the mixture was used as set forth in Example 21 in the form of a coating composition.

#### Example 24

Exemplifies the application of the process as set forth in Example 21 to mixtures of fixed oil and alkyd compounds with other substances:

A mixture of 25 parts alkyd resin (modified with soybean oil substance) with 10 parts melamine type resin (melamac resin) and 15 parts synthetic oil (derived from sorbitol with linseed fatty acids) was mixed with 18.5 parts toluene, 25 parts mineral spirit and 6.5 parts of butanol as solvents. To 100 parts thereof, 5 parts t-butyl hydroperoxide were added and the product was treated as set forth in Example 21 as a coating composition. Steel panels were dipped into the solution, allowed to drain and were exposed to a drying oven (120° C.). A well solidified and widely insolubilized film was obtained.

#### Example 25

Exemplifies the application of the process as set forth in Example 13 to a coating composition which contains pigments in addition to the soluble ingredients:

(a) A composition was obtained by mixing and milling together 1400 parts lead chromate, 680 parts red lead and 320 parts zinc oxide with 800 parts bodied linseed oil (Z-2) and 170 parts of petroleum naphtha solvent. Then 480 parts of

this paste were mixed with 300 parts of a 50% solution of soyabean oil-modified alkyd resin, 120 parts of 50% solution of a melamine type (melamac) resin and 325 parts toluene as thinner. To this composition, 5% t-butyl-hydroperoxide was added. This product was then used as a paint. It was applied as a coating and dried at about 130° C. A well-cured solvent resistant solidified coating was obtained.

(b) 89 parts commercial, standard Army olive-drab paint was thinned with 8.9 parts toluene and 2.22 parts t-butyl perbenzoate and the product was treated as in (a) above; a highly solidified, solvent resistant coating of high quality was obtained.

*Example 26*

This exemplifies the application of the present solidification process to a coating composition which contains at least a portion of fatty acid esters of polyhydroxyl alcohols, after such composition has been applied to another material.

100 feet of fiber glass covered electric wire were coated with a coating composition containing 50 parts of a commercial varnish produced at least partially from fatty acid esters of polyhydroxyl alcohols (in this example the varnish was based on a linseed oil composition dissolved in 50 parts mineral spirits). The wire was allowed to drain after being immersed in the varnish, and passed through an oven heated to 110° C. in 5 minute stages. The coating composition began to set, but had not been fully cured. Before curing had been completed, the wire was passed through a container holding a mixture of 10 parts tertiary butyl hydroperoxide in 30 parts petroleum naphtha. Alternatively, the liquid catalyst can be applied by dipping, spraying or the like. The coated catalyst treated wire was passed in 5 minute stages through an oven heated to 120° C., resulting in a well-cured, highly insolubilized coating.

*Example 27*

The catalyst, cumene hydroperoxide is a commercial product containing about 68.1% dimethyl-benzyl-hydroperoxide in dimethyl-benzyl alcohol and acetophenone, the actual hydroperoxide having a calculated active oxygen content of about 10%. 45 parts linseed oil were mixed with 5 parts commercial cumene hydroperoxide and 3 parts toluene. On heating, a vehement reaction occurred and the temperature went up to about 190° C. No solidification had occurred. The substance was allowed to cool to about 120° C. and 2 parts catalyst were added. On heating, solidification occurred rapidly. After boiling the reaction product in toluene, filtering and drying the solid substance, 38 g. or (89%) of the initial oil were obtained as a solidification.

*Example 28*

The solidification of fatty acid esters of resinous polyhydroxyl alcohols may also be accomplished by practice of the present invention as shown by the following example:

123 g. of a synthetic resinous polyhydroxyl alcohol, the condensation product of bis-phenol and epichlorohydrin (commercial Epon resin, in particular type No. 1004) were esterified by heating with 82.8 g. fatty acids. In this case, the chemically conjugated linseed fatty acids (commercial Conjuulin fatty acids) were used. The esterification was obtained in the usual manner by heating the compounds in an oil bath under continuous stirring and passing a flow of carbon dioxide

75

through the reaction vessel. Reaction was observed around 190° C. and the heating was continued to around 230° C. The resulting ester was a resin of a wax-like, milky appearance melting around 70° C.

To produce the solidification products in accordance with the present invention, 42 parts of the ester were melted with 6 parts toluene and 4 parts of t-butyl-perbenzoate catalyst. Three catalytic heating treatments were made, whereby solidification was obtained. The reaction product was purified by boiling twice in toluene, filtering and drying. 34 g. dry solidification were obtained.

*Example 29*

To exemplify the effect of the free oxygen action as procured from a substance which is capable of releasing such active oxygen, but which is not soluble in oil, hydrogen peroxide was used as follows:

(a) 47 g. bodied linseed oil were mixed with 15 grams 30% hydrogen peroxide and heated under stirring. Heavy foaming developed around 90° C. from the evaporation of the water and the oxygen release. Heating was continued up to 210° C. without solidification. After cooling to around 100° C., 10 g. hydrogen peroxide were added followed by heating up to 210° C. No solidification was obtained and after a third treatment with 9 g. hydrogen peroxide, solidification occurred. The solid particles were somewhat softer in texture than the other examples and swelled to a greater extent. They also exhibited a greater cohesive tendency than the solidifications from the previous examples. After heating twice with toluene, filtering and drying, 24 g. dry solids were obtained.

(b) 75 g. bodied linseed oil were heated in a vessel equipped with a mechanical stirrer. When the temperature reached about 90° C., the 30% hydrogen peroxide catalyst was allowed to drop continuously into the mixture. The first run was made with 25 g. peroxide. The water appeared to evaporate rapidly and gas development appeared to effect the oil under stirring. After the peroxide had been added, the temperature was allowed to raise and the reaction died down. Heating was discontinued at about 200° C. A slight gel was obtained. After resuming the heating of the mixture which had cooled off to about 95° C., peroxide was allowed to drop into the mixture under stirring. When about 15 g. peroxide had dropped in and the temperature had increased to about 120° C., solidification occurred to such an extent that movement of the mechanical stirrer was halted by the substance. The product was similar to that obtained in (a) above.

The present invention can be used for the production of the insolubilized form of fatty acid esters of polyhydroxyl alcohols and combinations of such esters with other ester-forming acids and compositions of such materials with other substances. Such products can be used as a stable, easily transportable and substantially resistant form of oil, wax, or fat products so long as it is not necessary to use these substances in liquid or soluble form.

The products of the present invention can also be separated from admixtures of the initial ester substances which do not take part in the actual solidification and which may be undesirable because of taste, odor or other undesirable qualities.

The solidified substances of the present in-

vention can be solubilized as set forth in my co-pending application Ser. No. 748,665 and can be used in the production of coatings, plastic compounds, etc. In this form of use, the present invention makes it possible to separate the part of the substance which is actually capable of solidification from other substances which are not capable of solidification, and combine such isolated products with other materials which are selected because of their characteristics, or to produce compounds which are more uniform than in their initial forms and which are therefore compatible with substances which are not compatible with the initial substance.

By applying this invention to solutions, it has become possible to produce coatings, impregnations, and similar compounds which can be stored, shipped and applied to the desired base in the desired form and which can then be insolubilized to a high degree of insolubilization.

By virtue of their easy form of handling, the catalysts themselves, or mixtures of the catalysts with other materials, can be kept separately and can be added to such compounds as intensifiers of the insolubilization at any time before ordering the actual application of the solution. They can also be used on previously applied and partially dried coatings, for further intensifying the insolubilization of the film, as by immersing the applied coating in the catalyst or to its combinations, and exposing such coated and immersed parts to conditions where the oxygen is freed directly on the coatings which are further to be solidified. Such immersion may be effected by dipping, spraying, etc. The coated substance, for instance long piece goods, like fabrics, cables, paper, etc. may be contacted by the free oxygen-yielding catalyst in a continuous process before completing the insolubilization of the coated materials.

A further aspect of my invention is that the processes and products disclosed and claimed hereby are adapted to be used in conjunction and cooperation with the processes and products disclosed and claimed in my copending application Ser. No. 748,665, now Patent 2,476,879, issued July 19, 1949. Briefly, this latter application relates to a process for solubilizing and liquifying fatty acid esters of alcohols, such as fixed oils, which are in a highly gelatinized state, by mixing them at elevated temperatures with a metal soap.

To avoid needless repetition in the present specification, I desire to state at this point that I have solubilized and liquified all the insolubilized, solidified products made in accordance with the foregoing working examples by utilizing the process of my aforesaid copending application. It is my intention that the aforesaid copending application be a part and parcel of the present specification to that extent and therefore my present application is a continuation-in-part of the aforesaid copending application Ser. No. 748,665, now Patent 2,476,879, issued July 19, 1949, in this respect.

In fact, the only process presently known to me for solubilizing and liquifying the solidified and insolubilized products of the present invention without decomposition is by use of my discovery as set forth in my aforesaid copending application.

It will be apparent that in this respect, my discoveries enable a complete and continuing cycle of physical transformations from a liquid, soluble state to a solidified, insoluble state and back

again, regardless of whether or not the materials treated at any stage of the transformation are in a non-gelatinized, partially-gelatinized or highly gelatinized form.

In the foregoing specification and working examples, I have selected a representative number of the many initial starting materials and oxygen-yielding catalysts which may be utilized with the process of my invention in order to obtain the novel resulting products. Among these compounds, all of which I intend to include within the scope of my appended claims, are the following:

Fatty acid esters of alcohols

From vegetable sources

Drying oils

Semi-drying and non-drying oils

Waxes and wax-like materials

From animal sources

Animal oils

Animal fats

Waxes and wax-like substances

From mineral sources

Montan wax

Synthetic oils and wax-like substances

Oil-modified alkyd resins

Fatty acids esters of resinous polyhydroxyl alcohols

Therefore, it will be apparent that by use of the term "fatty acid esters of alcohols," I mean to include both natural and synthetically produced compounds. In addition, I mean to include, monohydroxyl, dihydroxyl and other polyhydroxyl alcohols including resins and resinous polyhydroxyl alcohols. By use of the term "oils," I mean to include both natural and synthetic oils and fats and other lipids.

However, it will be apparent and understood that various modifications and equivalents coming within the realm of my discoveries may be used and I intend to include these within the scope of the appended claims defining my invention.

I claim:

1. A method of insolubilizing and solidifying higher fatty acid esters of alcohols characterized by their solubility in coal tar and petroleum solvents, which comprises treating said esters with at least about 4.5 percent by weight of an organic peroxide, at a temperature of at least about 90° C., and sufficiently elevated to effect substantially immediate and complete release of free oxygen therein to form a solidified reaction product in the form of a mass of incoherent, solid particles, said reaction product being insoluble in coal tar and petroleum solvents.

2. A method of insolubilizing and solidifying higher fatty acid esters of alcohols characterized by their solubility in coal tar and petroleum solvents, which comprises treating said esters with at least about 4.5 percent by weight of an alkyl peroxide, at a temperature of at least about 90° C., and sufficiently elevated to effect substantially immediate and complete release of free oxygen therein to form a solidified reaction product in the form of a mass of incoherent, solid particles, said reaction product being insoluble in coal tar and petroleum solvents.

3. A method of insolubilizing and solidifying higher fatty acid esters of alcohols characterized by their solubility in coal tar and petroleum solvents, which comprises treating said esters with at least about 4.5 percent by weight of an aryl peroxide, at a temperature of at least about 90°

19

C., and sufficiently elevated to effect substantially immediate and complete release of free oxygen therein to form a solidified reaction product in the form of a mass of incoherent, solid particles, said reaction product being insoluble in coal tar and petroleum solvents.

4. A method of insolubilizing and solidifying higher fatty acid esters of alcohols characterized by their solubility in coal tar and petroleum solvents, which comprises treating said esters with at least about 4.5 percent by weight of an alkyl-aryl peroxide, at a temperature of at least about 90° C., and sufficiently elevated to effect substantially immediate and complete release of free oxygen therein to form a solidified reaction product in the form of a mass of incoherent, solid particles, said reaction product being insoluble in coal tar and petroleum solvents.

5. The method set forth in claim 2 wherein the alkyl peroxide is an acetyl peroxide.

6. The method set forth in claim 2 wherein the alkyl peroxide is a butyl peroxide.

7. The method set forth in claim 3 wherein the aryl peroxide is a perbenzoate.

8. The method set forth in claim 3 wherein the aryl peroxide is a perphthalate.

9. The method set forth in claim 4 wherein the alkyl-aryl peroxide is a methylated benzoate.

10. A method of insolubilizing and solidifying higher fatty acid esters of monohydric alcohols characterized by their solubility in coal tar and petroleum solvents, which comprises treating said esters with at least about 4.5 percent by weight of an organic peroxide at a temperature of at least about 90° C., and sufficiently elevated to effect substantially immediate and complete release of free oxygen therein to form a solidified reaction product in the form of a mass of incoherent, solid particles, said reaction product being insoluble in coal tar and petroleum solvents.

11. A method of insolubilizing and solidifying higher fatty acid esters of polyhydric alcohols characterized by their solubility in coal tar and petroleum solvents, which comprises treating said

20

esters with at least about 4.5 percent by weight of an organic peroxide at a temperature of at least about 90° C., and sufficiently elevated to effect substantially immediate and complete release of free oxygen therein to form a solidified reaction product in the form of a mass of incoherent, solid particles, said reaction product being insoluble in coal tar and petroleum solvents.

12. The method set forth in claim 10 wherein the higher fatty acid ester of the monohydric alcohol is an ester-wax.

13. The method set forth in claim 10 wherein the monohydric alcohol is a high atomic alcohol.

14. The method set forth in claim 11 wherein the polyhydric alcohol is a glycol.

15. The method set forth in claim 11 wherein the polyhydric alcohol is a glycerol.

16. The method set forth in claim 1 wherein the higher fatty acid ester of an alcohol comprises a resin.

17. The method set forth in claim 1 wherein the higher fatty acid ester of an alcohol comprises a wax.

18. The method set forth in claim 1 wherein the higher fatty acid ester of an alcohol comprises an oil.

19. The method set forth in claim 1 wherein the higher fatty acid ester of an alcohol comprises a resinous fatty acid polyhydric alcohol ester of a condensation polymer of epichlorohydrin and bisphenol.

MAX KRONSTEIN.

#### REFERENCES CITED

35 The following references are of record in the file of this patent:

#### UNITED STATES PATENTS

| Number    | Name       | Date          |
|-----------|------------|---------------|
| 1,811,078 | Dykstra    | June 23, 1931 |
| 1,975,959 | Lawson     | Oct. 9, 1934  |
| 2,399,697 | Stark      | May 7, 1946   |
| 2,403,408 | Stamberger | July 2, 1946  |
| 2,442,330 | Fuller     | June 1, 1948  |